

## UNITED STATES PATENT OFFICE

2,658,003

## COATING COMPOSITION HAVING ACCELERATED DRYING TIME AND THE PROCESS OF ACCELERATING SAME

Louis E. Klein, St. Louis, Mo., and August R. Hempel, Dayton, Ohio, assignors to Monsanto Chemical Company, St. Louis, Mo., a corporation of Delaware

No Drawing. Application June 23, 1951,  
Serial No. 233,252

16 Claims. (Cl. 106—264)

1

This invention relates to new coating compositions comprising a drying vehicle and an improved drier therefor. More particularly the siccatives are polyvalent drier metal salts of monoalkyl esters of diisobutlenylsuccinic acid and triisobutlenylsuccinic acid, wherein the alkyl group contains from 1 to 4 carbon atoms, inclusive. More particularly still the drier metal is selected from the preferred group of polyvalent metals consisting of lead, cobalt, manganese, and zinc.

The prior art driers are resinates, linoleates and naphthenates of the polyvalent drier metals. The resinate and linoleate type driers oxidize very readily, becoming insoluble in the coating solvents and the drying vehicle, thus they must be used within a relatively short time after they are made. Also these driers may spontaneously ignite in storage and are accordingly a definite fire hazard. The naphthenates in general have improved solubilities and greater stability than the resinates and linoleates, but have an odor which is disagreeable to many consumers. In addition, the naphthenic acids are currently in short supply, pointing up the necessity of finding other suitable drier compositions.

One object of the present invention is to provide coating compositions which are characterized by faster drying properties. Another object of the present invention is to provide an improved drier which possesses good solubility in organic solvents employed in the coatings industry and in the drying vehicle. A further object is that the driers are substantially free of objectionable odors. Yet another object is to provide driers which are stable when exposed to oxidation conditions.

It has now been found that the polyvalent drier metal salts of monoalkyl esters of diisobutlenylsuccinic acid and triisobutlenylsuccinic acid with drying vehicles provides an improved coating composition which has faster drying properties than with conventional commercial driers, and the drier is characterized by good solubility in coating solvents and drying vehicles; is exceptionally stable against oxidation, notwithstanding the presence of the alkenyl group; is substantially free of any disagreeable odor; and is capable of volume production from available raw materials.

2

By the term "polyvalent drier metal" it is understood that the conventional driers are meant. The preferred drier metals are lead, cobalt, manganese and zinc, but other metals, such as aluminum, calcium, cerium, chromium, copper, iron, nickel, and vanadium may also be employed. The latter metals are not as active as the former group, but are often beneficially employed therewith for special effects and are accordingly within the scope of this invention. Thus, mixed driers are also understood to be within the scope of this invention.

In general the conventional quantities of the driers, reported as weight per cent of metal based on the weight of the drying vehicle solids, are employed. Thus, preferably from about 0.2 to about 0.5 per cent of lead is generally used, although up to 2.0 per cent and even higher may be incorporated for special effects. The surface-drying metals, cobalt and manganese, are normally used within a range of from about 0.01 to about 0.1 per cent, but here too higher quantities may be employed for specific results as, for example, the production of a wrinkle finish.

The term "drying vehicle" is employed herein to mean a fluid organic composition which sets by oxidation and polymerization, as for example, drying oils, paints, lacquers, enamels, varnishes, styrenated alkyds and similar resinous coating materials.

The driers are prepared for use by dissolving in a conventional solvent, as for example, mineral spirits, V. M. and P. naphtha, xylene, toluene and benzene. Concentrated solutions containing more than 50 per cent solids can be prepared, as for example, cobalt monomethyl diisobutlenylsuccinate in mineral spirits.

The following examples are illustrative of the invention:

## Example 1

A long linseed oil modified phthalic anhydride-pentaerythritol alkyd resin having a viscosity of  $\gamma$  at 70 per cent solids in mineral spirits was further cut to about 50 per cent solids with additional mineral spirits. To two samples of the aforesaid resin 0.02 weight per cent of metal based on the weight of the alkyd resin solids of a cobalt drier was added. Sample A contained cobalt naphthenate and sample B contained cobalt monomethyl diisobutlenylsuccinate. The

samples were aged briefly and then applied as a 0.002 inch film on tin. Sample B comprising the composition of this invention was set in less than three hours whereas sample A was not set for a substantially greater period of time. It was particularly noted that the drier of sample B had no odor as compared to the cobalt naphthenate drier.

*Example 2*

A sample of bodied linseed oil was cut to about 70 per cent solids with mineral spirits. To each of two samples thereof 0.04 per cent based on the oil cobalt drier was added, sample A being cobalt naphthenate and sample B being cobalt monomethyl diisobutlenylsuccinate. The two samples were then coated on tin panels and tested periodically. Sample B set dust-free in about 5.5 hours, whereas sample A was not dust-free after this period of time.

*Example 3*

A long soybean oil modified phthalic anhydride-pentaerythritol alkyl resin was cut to about 50 per cent solids by the addition of mineral spirits. To two samples of the above cobalt naphthenate (A) and cobalt monomethyl diisobutlenylsuccinate (B) were added, respectively, such that 0.05 per cent of the cobalt drier based on resin solids was employed. Sample B was set in about 2 hours, dust-free in less than about 3 hours, and tack-free in less than about 5 hours; whereas, sample A required, respectively, about 3 hours, less than 4 hours, and was not yet tack-free after about 5 hours.

*Example 4*

To five samples of castor oil modified phthalic anhydride-glycerol alkyl resin, cut to 38 per cent solids with mineral spirits, 0.04 per cent of a cobalt drier based on resin solids was added as follows:

Sample A—Cobalt naphthenate

Sample B—Cobalt monomethyl diisobutlenylsuccinate

Sample C—Cobalt monoisopropyl diisobutlenylsuccinate

Sample D—Cobalt monobutyl triisobutlenylsuccinate

Sample E—Cobalt octoate

Sample B was found to set and become dust-free faster than the other samples, sample D was slightly faster than A and E, and sample C required a slightly greater time than A and E.

Other driers which can be employed are for example:

Lead monoethyl diisobutlenylsuccinate

Zinc monopropyl diisobutlenylsuccinate

Manganese monoisobutyl diisobutlenylsuccinate

Lead monomethyl triisobutlenylsuccinate

Zinc monoethyl triisobutlenylsuccinate

Manganese monoisopropyl triisobutlenylsuccinate

The drier metal salts, for example, cobalt, manganese, and lead salts of diisobutlenylsuccinic and triisobutlenylsuccinic acids were found to be useless as driers in that they were insoluble in coating solvents and accordingly failed to meet one of the major requirements of a drier. The monoalkyl esters of the aforesaid acids containing more than four carbon atoms also have poor solubility and the progressively smaller weight ratio of the drier metal to the molecular weight of the compounds also is detrimental.

**We claim:**

1. A coating composition comprising a drying vehicle and an effective amount up to about 2 per cent by weight of metal, based on the weight of the drying vehicle solids, of a drier comprising a polyvalent drier metal salt of the monoalkyl esters of diisobutlenylsuccinic acid and triisobutlenylsuccinic acid, wherein the alkyl group contains from 1 to 4 carbon atoms, inclusive.

2. A coating composition comprising a drying vehicle and an effective amount up to about 2 per cent by weight of metal, based on the weight of the drying vehicle solids, of a drier comprising a drier metal salt of the monoalkyl esters of diisobutlenylsuccinic acid, wherein the drier metal is selected from the group consisting of lead, cobalt, manganese, and zinc and mixtures thereof, and the alkyl group contains from 1 to 4 carbon atoms, inclusive.

3. A coating composition comprising a drying vehicle and an effective amount up to about 2 per cent by weight of metal, based on the weight of the drying vehicle solids, of a drier comprising a drier metal salt of the monoalkyl esters of triisobutlenylsuccinic acid, wherein the drier metal is selected from the group consisting of lead, cobalt, manganese, and zinc and mixtures thereof, and the alkyl group contains from 1 to 4 carbon atoms, inclusive.

4. A coating composition comprising a drying vehicle and an effective amount up to about 2 per cent by weight of metal, based on the weight of the drying vehicle solids, of cobalt monomethyl diisobutlenylsuccinate.

5. A coating composition comprising a drying vehicle and an effective amount up to about 2 per cent by weight of metal, based on the weight of the drying vehicle solids, of cobalt monoisopropyl diisobutlenylsuccinate.

6. A coating composition comprising a drying vehicle and an effective amount up to about 2 per cent by weight of metal, based on the weight of the drying vehicle solids, of cobalt monobutyl triisobutlenylsuccinate.

7. A coating composition comprising a drying vehicle and an effective amount up to about 2 per cent by weight of metal, based on the weight of the drying vehicle solids, of lead monomethyl diisobutlenylsuccinate.

8. A coating composition comprising a drying vehicle and an effective amount up to about 2 per cent by weight of metal, based on the weight of the drying vehicle solids, of manganese monomethyl diisobutlenylsuccinate.

9. The process of accelerating the set of a drying vehicle, which comprises mixing with the drying vehicle an effective amount up to about 2 per cent by weight of metal, based on the weight of the drying vehicle solids, of a polyvalent drier metal salt of the monoalkyl esters of diisobutlenylsuccinic acid and triisobutlenylsuccinic acid, wherein the alkyl group contains from 1 to 4 carbon atoms, inclusive.

10. The process of accelerating the set of a drying vehicle, which comprises mixing with the drying vehicle an effective amount up to about 2 per cent by weight of metal, based on the weight of the drying vehicle solids, of a drier metal salt of the monoalkyl esters of diisobutlenylsuccinic acid, wherein the drier metal is selected from the group consisting of lead, cobalt, manganese, and zinc and mixtures thereof, and the alkyl group contains from 1 to 4 carbon atoms, inclusive.

11. The process of accelerating the set of a drying vehicle, which comprises mixing with the

drying vehicle an effective amount up to about 2 per cent by weight of metal, based on the weight of the drying vehicle solids, of a drier metal salt of the monoalkyl esters of triisobutlenylsuccinic acid, wherein the drier metal is selected from the group consisting of lead, cobalt, manganese, and zinc and mixtures thereof, and the alkyl group contains from 1 to 4 carbon atoms, inclusive.

12. The process of accelerating the set of a drying vehicle, which comprises mixing with the drying vehicle an effective amount up to about 2 per cent by weight of metal, based on the weight of the drying vehicle solids, of cobalt monomethyl diisobutlenylsuccinate.

13. The process of accelerating the set of a drying vehicle, which comprises mixing with the drying vehicle an effective amount up to about 2 per cent by weight of metal, based on the weight of the drying vehicle solids, of cobalt monoisopropyl diisobutlenylsuccinate.

14. The process of accelerating the set of a drying vehicle, which comprises mixing with the drying vehicle an effective amount up to about 2

per cent by weight of metal, based on the weight of the drying vehicle solids, of cobalt monobutyl triisobutlenylsuccinate.

15. The process of accelerating the set of a drying vehicle, which comprises mixing with the drying vehicle an effective amount up to about 2 per cent by weight of metal, based on the weight of the drying vehicle solids, of lead monomethyl diisobutlenylsuccinate.

16. The process of accelerating the set of a drying vehicle, which comprises mixing with the drying vehicle an effective amount up to about 2 per cent by weight of metal, based on the weight of the drying vehicle solids, of manganese monomethyl diisobutlenylsuccinate.

LOUIS E. KLIEN.  
AUGUST R. HEMPEL.

## References Cited in the file of this patent

20

## UNITED STATES PATENTS

| Number    | Name    | Date          |
|-----------|---------|---------------|
| 2,380,699 | Kyrides | July 31, 1945 |